# EUROPEAN PATENT SPECIFICATION

(11) **EP 0 179 952 B1**
(45) Date of publication and mention of the grant of the patent: **14.09.1988**
(21) Application number: 84201584.4
(22) Date of filing: 30.10.1984
(51) Int. Cl.: C21D 8/02, C21D 7/13

(54) **Method for producing high strength steel with good ductility**
Verfahren zur Herstellung von hochfestem und duktilem Stahl
Procédé pour la fabrication d'acier à haute résistance mécanique et présentant une bonne ductilité

(43) Date of publication of application: 07.05.1986
(73) Proprietor: SSAB Svenskt Stal AB, S-103 26 Stockholm (SE)
(72) Inventor: Josefsson, Erik Anders Ake, S-781 52 Borlänge (SE)
(74) Representative: Wärulf, Olov

(56) References cited:
- EP-A- 0 098 564
- DE-A- 2 037 350
- US-A- 3 849 209
- US-A- 4 400 223

## Description

### Technical area

The present invention relates generally to a method for fabricating structural steel which has high strength and good ductility. _{'}

### Technical background

In the conventional fabrication of structural steel such that the steel has both high strength and good ductility (low transition temperature), small additions of the so-called grain refining element (Nb, V, Ti, B) have been used to a great extent along with a method of hot rolling the steel where the reductions in the individual passes as well as the deformation temperatures are regulated with respect to the structure desired. This method is often termed controlled rolling. The objective of the controlled rolling method is that when the rolling is completed, either a fine-grained recrystallized austenite or a heavy deformed unrecrystallized austenite structure has been produced in the steel.

The former structure is obtained by making the finishing rolling passes with a high degree of reduction, the latter structure by effecting the finishing rolling passes at a low temperature i.e., at a temperature lower than about 900°C. It is the fine grain of the recrystallized austenite, and in the alternative, the high degree of reduction of the non-recrystallized austenite that provide the basis for forming a fine-grained polygonal ferrite during the subsequent cooling, and thus a basis for the combination of the high strength and good ductility characteristics of the finished steel.

To obtain a fine grained ferrite after the first alternative of controlled rolling where a fine grained recrystallized austenite is produced after the last pass, it is necessary not only that the steel contains a suitable amount of grain-refining elements, e.g. Nb, but, also that at least in this last pass, reduction is relatively high, i.e., with an area reduction of 30% or more, as the recrystallized grain size of the austenite which is within the range of interest here, uniformly decreases with increasing reduction. On the other hand, in the last stage of the rolling, it is advisable to avoid reductions about and below about 20% as at this point, according to known laws for recrystallization, as there is a risk of producing enlarged recrystallized grains when approaching the so-called critical draft (degree of reduction). At even lower reductions, grain-coarsening has appeared even in grains without recrystallization by the so-called strain induced grain growth. With several such light passes, there also appears a risk for partial recrystallization and the known phenomenon of non-uniform grain size, which means a large loss of ductility and strength for the steel.

The other method mentioned above, where the rolling is conducted such that recrystallization does not occur, requires that, after a certain degree of roughening, the material must be cooled to a temperature below about 900°C, normally below about 850°C, before the finish rolling begins which causes retained deformation of the austenite. This method is often characterized as a thermomechanical treatment.

Both methods set forth above have inherent disadvantages with respect to the technical portion of the rolling procedure. High reductions during the finishing pass according to the first method require high roll forces which means that the capacity of the rolling mill can be a limiting factor. In addition, it is more difficult to maintain narrow thickness tolerances with high reductions. Another aggravating circumstance is that, to obtain good results in the form of fine grain in the final structure, the finishing temperature must be kept fairly low, as other conditions being equal, the recrystallized grain size becomes finer, the lower the deformation temperature is, and a low rolling temperature also contributes to an increase in the roll load. Conducting the rolling within the temperature range for non-recrystallization also results in extra loads in the rolling mill and is also an impediment for material flow since the material has to cool between roughening and the finishing rolling which increases the fabrication time and also decreases rolling capacity.

### Description of the invention

In accordance with the method of the present invention, it has now been shown, however, that, even with small finishing reductions under certain circumstances, it is possible to obtain steel with equal or better properties as compared with a high finishing reduction and this method can be accomplished without delaying the rolling by utilizing the low finishing temperatures which are required in the second rolling sequence as described above. The finish rolling can, on the contrary, be conducted directly after roughening in the temperature range of about 900 to 1100°C and with low reductions, i.e., below about 15%.

Thus, the present invention provides a method for producing hot rolled steel products having high strength and ductility. The method consists in a process for manufacturing hot rolled steel products having high strength and good ductility as hot rolled, the method comprising heating and low-alloy steel having a C content within the range of about 0.02 to 0.15 wt% a Nb content within the range of about 0.015 to 0.100 wt% and a titanium content within the range of about 0.005 to 0.040 wt% to a temperature in the range of about 1150 to 1250°C, hot rolling the steel in one or more passes during a first rolling sequence such that the average austenite grain size is reduced to below 50 J.lm at the end of the first sequence, the first sequence being completed with, the steel at a temperature in the range of about 950 to 1100°C, directly thereafter hot rolling the steel at about 9000 to 1100°C in a second rolling sequence of one or more passes, the reduction in each pass being below about 15%, and cooling the steel to ambient temperature.

The method of the invention is explained in further detail in the following with reference to the drawing in which the sole figure is a graphical representation of the mechanical properties of various steels, some of the steels having been produced by the method of the invention and others by methods outside the scope of the invention.

More particularly, in the method of the invention, the steel should contain a certain amount of Nb, e.g., about 0.015 to about 0.100%, the lower amount applicable to higher carbon contents, e.g., about .15% C and the higher amount applicable to a carbon content of about 0.05% and lower. Generally, the steels particularly suitable for the method, contain minor amounts, e.g., less than about 2%, of one or more of Si, Mn, Cr and Mo.

In the present invention, the rolling of the steel is divided into two sequences. The first sequence is conducted such that the steel has a uniform, relatively fine grained recrystallized austenite (average less than 50 J.lm measured on a sample section which has been cut out and water quenched) at the end of the sequence. To achieve this structure, at least in the last pass in this first sequence, the area reduction oftentimes exceeds about 25%, preferably about 30%. The second rolling sequence includes one or more light passes, each pass producing less than about 15% in area reduction. This second sequence can immediately following the first sequence without any time waiting for the steel to cool if the temperature of the heat at the end of the first sequence is below about 1100°C, and for lower amounts of Nb, below about 1070°C.

To achieve the desired uniform, relatively fine grained austenite at the end of the first rolling sequence, it has been found to be advantageous to include Ti in amounts between about 0.005 and about 0.04%.

Furthermore, when particularly good ductility in the steel is required, it has proven important that at least one of the light finishing passes be conducted at a sufficiently high temperature (about 950° to 1100°C) so that the precipitation of NbC from the austenite is favored as much as possible. Since the austenite obtained by the procedure of light finishing passes tends to transform to ferrite more readily as compared with the same austenite rolled by conventional methods, the procedure of the invention is well adapted to be combined with accelerated cooling by water spraying and the like as an extra strength increasing step performed after the second rolling sequence.

The steel produced by the method of the invention is compared to steel produced by methods outside the scope of the invention in the following example.

### Example

A number of steel blooms with the approximate analysis of 0.09% C, 0.33% Si, 1.41% Mn, 0.013% P, 0.011 % S, 0.010% N, 0.027% Al, 0.007% Ti and 0.027% Nb were heated to about 1200°C and hot rolled from a thickness of about 120 mm to a thickness of about 20 mm as per the different pass schedules set forth in the following table. When passing from the first rolling sequence with high degrees of reduction to the second rolling sequence with ligh passes, the temperature of the plate bar was determinsd and sample sections were cut and cooled in water. In each of the sample sections, the austenite grain size existing before the cooling was determined. After the finish rolling of the second sequence, the plates were allowed to cool in air. The mechanical properties of the plates were determined from test bars that were cut normal to the rolling direction. The test results are set forth in the upper portion of the Table.

In another rolling series, blooms from the same heat as in earlier series were heated to about 1170°C. Hot rolling was performed and, as was done previously, the reductions for the particular passes were varied. The test results from this series are set forth in the lower portion of the Table. For greater clarity, the most important property values, i.c., the yield point and the transition temperature, are graphically presented in the drawing.

From the results set forth in the Table and the Drawing it can be noted that the plates with low reductions in the second rolling sequence show a better combination of yield point and transition temperature characteristics than the plates produced with high reductions, such as 35% in the finishing pass. It should also be noted that, with a reduction of 17% in the finishing pass (plate 0), a lower ductility is obtained than in the plates where finishing reductions are limited to below about 15%. A lower ductility is also obtained after the normal rolling with high finishing reduction of 35% (plates D and K).

To the extent not indicated, all percentages set forth above are by weight.

## Claims

1. A process for manufacturing hot rolled steel products having high strength and good ductility as hot rolled, the method comprising heating a low-alloy steel having a C content within the range of about 0.02 to 0.15 wt%, a Nb content within the range of about 0.015 to 0.100 wt% and a titanium content within the range of about 0.005 to 0.040 wt% to a temperature in the range of about 1150 to 1250°C, hot rolling the steel in one or more passes during a first rolling sequence such that the average austenite grain size is reduced to below 50 pm at the end of the first sequence, the first sequence being completed with the steel at a temperature in the range of about 950 to 1100°C, directly thereafter hot rolling the steel at about 900° to 1100°C in a second rolling sequence of one or more passes, the reduction in each pass being below about 15%, and cooling the steel to ambient temperature.

2. A process according to claim 1, wherein the reduction in the last pass of the first rolling sequence exceeds about 25%.

3. A process according to claim 1, wherein the reduction in the last pass of the first rolling sequence exceeds about 30%.

4. A process according to claim 1, wherein during at least one of the passes in the second rolling sequence, the temperature of the steel is in the range of about 1100 to 950°C.

5. A process according to claim 1 or 4, wherein the cooling after the second rolling sequence is accelerated by water spraying.

6. A process according to claim 1, wherein the steel contains less than 2 wt% of one or more of Si, Mn, Cr and Mo.

## Patentansprüche

1. Verfahren zur Herstellung warmgewalzter Stahlprodukte mit hoher Festigkeit und guter Streckbarkeit beim Warmwalzen, wobei beim Verfahren ein niedrig ligierter Stahl mit einem C-Gehalt im Bereich von etwa 0,02 bis 0,15 Gew.%, einem Nb-Gehalt im Bereich von etwa 0,015 bis 0,100 Gew.% und einem Ti-Gehalt im Bereich von etwa 0,005 bis 0,040 Gew.% auf eine Temperatur im Bereich von etwa 1150 bis 1250°C erwärmt wird, der Stahl in einem oder mehreren Durchgängen während einer ersten Walzreihe warmgewalzt wird, so daß die mittlere Austenitkorngröße auf kleiner 50 um am Ende der ersten Reihe verringert wird, nach Beendigung der ersten Reihe der Stahl bei einer Temperatur im Bereich von etwa 950 bis 1100°C ist, worauf unmittelbar danach der Stahl bei etwa 900 bis 1100°C in einer zweiten Walzreihe von einem oder mehreren Durchgängen warmgewalzt wird und die Verringerung bei jedem Durchgang unter etwa 15% liegt und der Stahl bei Raumtemperatur gekühlt wird.

2. Verfahren nach Anspruch 1, bei dem die Verringerung beim letzten Durchgang der ersten Walzreihe etwa 25% überschreitet.

3. Verfahren nach Anspruch 1, bei dem die Verringerung beim letzten Durchgäng der ersten Walzreihe etwa 30% überschreitet.

4. Verfahren nach Anspruch 1, bei dem während wenigstens einem Durchgang der zweiten Walzreihe die Temperatur des Stahles im Bereich von etwa 1100 bis 950°C ist.

5. Verfahren nach Anspruch 1 oder 4, bei dem das Kühlen nach der zweiten Walzreihe durch Wassersprühung beschleunigt wird.

6. Verfahren nach Anspruch 1, bei dem der Stahl weniger als 2 Gew.% einer oder mehrerer der Substanzen Si, Mn, Cr und Mo enthält.

## Revendications

1. Procédé de fabrication de produits en acier laminé à chaud ayant une résistance élevée et une bonne ductilité sous la forme laminée à chaud, le procédé comprenant le chauffage d'un acier faiblement allié ayant une teneur en C comprise dans le domaine d'environ 0,02 à 0,15% en poids, une teneur en Nb comprise dans le domaine d'environ 0,015 à 0,2% en poids et une teneur en titane comprise dans le domaine d'environ 0,005 à 0,040% en poids à une température comprise dans le domaine d'environ 1 150 à 1 250°C, le laminage à chaud de l'acier en une ou plusieurs passes au cours d'une première séquence de laminage telle que la dimension moyenne des grains d'austénite est réduite jusqu'à moins de 50 pm à la fin de la première séquence, la première séquence étant complétés ensuite directement l'acier étant à une température dans le domaine d'environ 950 à 1 100°C, par un laminage à chaud de l'acier à environ 900 à 1 100°C dans une deuxième séquence de laminage à une ou plusieurs passes, la réduction à chaque passe étant inférieure à environ 15%, et le refroidissement de l'acier jusqu'à la température ambiante.

2. Procédé selon la revendication 1, dans lequel la réduction dans la dernière passe de la première séquence de laminage dépasse environ 25%.

3. Procédé selon la revendication 1, dans lequel la réduction dans la dernière passe de la première séquence de laminage dépasse environ 30%.

4. Procédé selon la revendication 1, dans lequel au cours d'au moins l'une des passes de la deuxième séquence de laminage, la température de l'acier est dans le domaine d'environ 1 100 à 950°C.

5. Procédé selon la revendication 1 ou 4, dans lequel le refroidissement après la deuxième séquence de laminage est accéléré par une aspersion d'eau.

6. Procédé selon la revendication 1, dans lequel l'acier contient moins de 2% en poids d'un ou de plusieurs des éléments Si, Mn, Cr, et Mo.
